

1

3,560,384

ASHLESS LUBRICANT ADDITIVE  
 Robert A. Halling, Wilmington, Del., assignor to E. I. du  
 Pont de Nemours and Company, Wilmington, Del., a  
 corporation of Delaware  
 No Drawing. Filed Oct. 14, 1968, Ser. No. 767,486  
 Int. Cl. C10m 1/48  
 U.S. CL. 252—46.7

5 Claims

ABSTRACT OF THE DISCLOSURE

An ashless lubricant additive which improves the viscosity index, the anti-corrosion, anti-oxidant, anti-wear and detergent properties of the base oil. The additive is the reaction product of

(A) a phosphosulfurized ethylene/propylene/1,4-hexadiene terpolymer having an average molecular weight of between about 3,500 and about 65,000 and containing about 35–70 weight percent propylene, about 1–6 weight percent 1,4-hexadiene and the remainder being ethylene; with

(B) an amine of the formula



wherein  $x$  is an integer of 2 or 3, and R and  $R_1$  are alkyl groups of 1–4 carbon atoms.

BACKGROUND OF THE INVENTION

(1) Field of the invention

This invention relates to an ashless lubricant additive, and more particularly to the product of an amine and a phosphosulfurized olefin terpolymer.

(2) Description of the prior art

Ashless lubricant additives comprising the reaction product obtained by (a) treating polyisobutylene or polypropylene, with  $\text{P}_2\text{S}_5$ , (b) hydrolyzing the olefin- $\text{P}_2\text{S}_5$  product, and (c) treating the hydrolyzed product with an aliphatic amine or an alkylene polyamine have been found useful in improving the dispersancy of lubricating oils and in improving the detergent properties of the lubricating oil (see U.S. 3,143,506).

More recently, an ashless lubricant additive was prepared comprising the reaction product obtained by (a) treating a low-molecular-weight polyisobutylene (mol. wt. 250–1500) with  $\text{P}_2\text{S}_5$  and (b) reacting the phosphosulfurized polyisobutylene with an amine of the formula



wherein  $x$  is 1–9 (see U.S. 3,329,612). These lubricant additives are described as improving the anti-corrosion, anti-oxidant and anti-wear properties of the lubricating oil as well as improving the oil's detergent properties.

However, it is sometimes necessary to add a viscosity index improver to lubricating oils containing the above-described ashless lubricant additives, inasmuch as the above-described additives do not improve the viscosity-temperature characteristics of the oils to any extent.

Accordingly, it is an object of this invention to provide an ashless lubricant additive which improves the viscosity index of the lubricating oil as well as improving the detergent, anti-corrosion, anti-oxidant and anti-wear properties. This and other objects will be apparent as hereinafter described.

In addition to improving the viscosity index of lubricating oils, the additives of this invention have been found to unexpectedly improve the performance of ex-

2

treme pressure additives in a compounded lubricating oil, even though they do not possess extreme pressure properties themselves. Moreover, the additives of this invention possess exceptionally high shear stability.

SUMMARY OF THE INVENTION

This invention is directed to a lubricant additive comprising the product obtained by reacting

(A) A phosphosulfurized ethylene/propylene/1,4-hexadiene terpolymer having an average molecular weight of between about 3,500 and about 65,000 and containing about 35–70 weight percent propylene, about 1–6 weight percent 1,4-hexadiene and the remainder being ethylene; with

(B) An amine of the formula



wherein  $x$  is an integer of 2 or 3, and R and  $R_1$  are alkyl groups of 1–4 carbon atoms.

The invention is also directed to a lubricant composition of a mineral lubricating oil and from about 0.1 to about 4 percent by weight of the oil of the additive defined in the preceding paragraph.

The invention is further directed to a lubricant additive concentrate comprising a neutral lubricating oil and about 5 to about 50 percent by weight of the oil of the additive defined in the first paragraph of this summary.

DESCRIPTION OF THE INVENTION

The lubricant additive of this invention is conveniently prepared by a two-step process.

The first step comprises reacting the ethylene/propylene/1,4-hexadiene terpolymer with  $\text{P}_2\text{S}_5$  in the substantial absence of oxygen and under essentially anhydrous conditions, e.g., in an atmosphere of nitrogen or other inert gases, at a temperature of between about 200° F. and 500° F. The amount of  $\text{P}_2\text{S}_5$  employed is ordinarily between about 0.25 to about 5 moles per mole of 1,4-hexadiene in the terpolymer. Preferably 0.5 to 1.5 moles of  $\text{P}_2\text{S}_5$  are used. The time of reaction is normally between about 4 and about 30 hours. The use of an inert solvent, e.g., a hydrocarbon such as hexane, octane, or a halocarbon such as 1,2,4-trichlorobenzene is desirable. A halocarbon such as a chloroaromatic compound is preferred.

The second step comprises reacting the phosphosulfurized terpolymer, which can be used after merely decanting or filtering the reaction mass of the first step to remove insoluble byproducts and unreacted reactants, with the amine. The second step is carried out at a temperature of between about 200° F. and about 500° F. for a period of about 4 to about 30 hours. The amount of the amine employed can range between about 2 to about 6 moles of amine per atom of phosphorus employed in the first step. The preferred amount of amine used is between 2 and 4 moles per atom of phosphorus. The same or a different solvent as used in the first step can be employed in this second step. When the same solvent is used in both steps the reaction mass of the first step can be employed directly. The final product is ordinarily isolated by usual methods, as for example by precipitating with methanol. However, if the solvent employed in the reaction sequence is compatible with the lubricating oil, the final mixture need only be filtered, or at most, needs only a water wash followed by drying. The product, if isolated, may be purified by extraction with methanol, followed by drying.

The pressure employed in the reaction is preferably atmospheric, although super- or subatmospheric pressures may be used.

The terpolymers employed in the composition of this invention are amorphous polymers which can contain 35-70 weight percent propylene, 1-6 weight percent 1,4-hexadiene with the remainder ethylene. Preferred weight percent ranges are 42-55 weight percent propylene, 1-4 weight percent 1,4-hexadiene with the remainder ethylene. Preferably the terpolymers should have a relatively narrow molecular weight distribution. The molecular weight distribution, which is determined by dividing the weight average molecular weight by the number average molecular weight, should be less than 8.

Suitable copolymers are the essentially amorphous, oil soluble copolymers of ethylene which are prepared by polymerization in the presence of coordination catalysts. Polymerization with these catalysts is well known, as described, for example, in U.S. 2,799,668, 2,975,159 and 2,933,480. Since the utilization of these catalysts can produce a variety of polymers from ethylene and propylene, it is important to control the conditions of the reaction in order to obtain the specific amorphous polymers useful in the invention having specified molecular weights and a narrow molecular weight distribution.

More specifically, in order to obtain the amorphous copolymers desired, it is advantageous to use a hydrocarbon soluble vanadium compound, e.g.  $\text{VOCl}_3$  or vanadium triacetylacetone, in combination with an alkyl aluminum chloride as described by Natta et al. in U.S. 3,300,459 and in J. Polymer Sci., 51, 411ff and 429ff (1961). Use of this catalyst system results in essentially amorphous copolymers soluble in a mineral lubricating oil. Such copolymers exhibit substantially no crystallinity as evidenced by X-ray examination.

The effectiveness of the subject copolymers as viscosity index improvers lies also in the controlled molecular weight range and narrow distribution of the molecular weight. This can be achieved by methods described by Natta in J. Polymer Sci., 34, 541ff (1959), e.g. by the use of chain transfer agents such as metal alkyls, esp. zinc alkyls, and by use of hydrogen pressure, U.S. 3,051,690. The article by Natta above cited, J. Polymer Sci., 51, 411 (1961), also described the operative conditions for the preparation of such polymers, such as time, temperature, catalyst concentration and monomer concentration.

As is well known, these catalysts must be used in strict absence of oxygen, water or other material with which they react. For this reason the solvents in which they are used are greatly limited, the preferred ones being the saturated aliphatic and hydroaromatic hydrocarbons and certain nonreactive halogen compounds such as tetrachloroethylene and chlorobenzenes. These compounds conveniently serve as solvents for the polymerization which is usually carried out in a dilute suspension of the catalyst. The polymerization is normally carried out at ordinary temperatures and pressures.

The inherent viscosity range of the terpolymer is between about 0.1 and 1 as measured as a 0.1 weight percent solution in tetrachloroethylene at 30° C. The range of 0.1 to 1.0 corresponds to about 3,500 to 65,000 weight average molecular weight as determined by light scattering. Preferred terpolymers have an inherent viscosity of 0.1 to 0.6, correspond to 3,500 to 35,000 weight average molecular weight.

Amines suitable for use in this invention are those of the formula



wherein  $x$  is 2 or 3 and R and  $R_1$  are the same or different alkyl groups of 1-4 carbon atoms. Preferably R and  $R_1$  are the same. Representative suitable amines include N,N-dimethyl-1,3-propanediamine, N,N-dimethylethylenediamine, N,N-diethyl-1,3-propanediamine, N,N-diethylethylenediamine, N,N-dipropyl-1,3-propanediamine, N,N-di-

propylethylenediamine, N,N-dibutyl-1,3-propanediamine, N,N-dibutylethylenediamine, and the like.

The reaction product formed as described previously does not have a definite stoichiometric relationship between the phosphorus, sulfur and nitrogen atoms present. Hence the reaction product of this invention is believed to be a mixture of products.

The reaction product is useful, as stated previously, as an additive for improving the properties of mineral or neutral lubricating oils, such as crankcase oils, automotive transmission fluid base oils or hydraulic fluid base oils. Lubricating oils and transmission fluids are predominantly paraffinic, solvent-refined neutral oils having Saybolt Universal Seconds (S.U.S.) viscosities of about 60 to 220 at 100° F. and viscosity indices of about 80 to 110. For use with the additives of this invention, preferred lubricating oils should have S.U.S. viscosities of about 90 to 160, while preferred transmission fluids should have S.U.S. viscosities of about 60 to 110. Hydraulic fluid base oils are predominantly naphthenic, solvent-refined neutral oils having S.U.S. viscosities of not greater than about 50 and pour points not over —65° F.

Effective amounts of the additive of this invention are employed with the mineral or neutral oils, usually between about 0.1 to 4 percent by weight of the oil and preferably between about 1-3 percent. The additive may be incorporated into the oil by first milling or blending the additive in a small portion of the base oil to form a concentrate containing between about 5 and about 50 percent of the additive by weight based on the weight of base oil. The concentrate is then blended into the oil to the desired effective concentration of additive. Preferred base oils for use in forming the concentrates are the paraffinic, naphthenic or mixed neutral oils of 70 to 150 S.U.S. viscosity at 100° F. If desired, solution time may be decreased by preheating the oil to 170-210° F. before milling or blending.

The following examples describe the preparation of the additives and their usefulness in greater detail, and are meant to be representative rather than limiting. All parts are by weight unless otherwise indicated.

#### EXAMPLE A

A typical terpolymer preparation is as follows: Ethylene, propylene and 1,4-hexadiene are polymerized in an evaporatively cooled, continuous flow, stirred reactor operated at 30° C. The partial pressures and flow rates of the monomers are adjusted to obtain the desired composition. The terpolymers used in the examples which follow were made in hexane solution in the presence of a coordination catalyst formed in situ by combining diisobutyl aluminum monochloride with vanadium tris(acetylacetone). The partial pressure of hydrogen in the reactor was 15.6 lb./sq. in. (absolute) and the residence time was 36.3 minutes.

#### EXAMPLE 1

##### Preparation of additive

In 1800 ml. of 1,2,4-trichlorobenzene with a dry nitrogen atmosphere about it were reacted 100 g. (0.043 mole as 1,4-hexadiene) of an ethylene, propylene, 1,4-hexadiene terpolymer having a wt. ratio of E-61.7/P-34.9/HD-3.4 and an inherent viscosity of 0.44 (as measured on a 0.1 wt. percent solution in tetrachloroethylene at 30°, about 23,000 mol. wt.) and 20 g. (0.09 mole)  $\text{P}_2\text{S}_5$  at a temperature of 200-210° C. for a period of 6 hours. The reaction mixture was cooled and the insoluble residue was removed by decanting the solution. To the solution was added 51 g. (0.5 mole) N,N-dimethyl-1,3-propanediamine. The temperature was raised slowly to 205-210° C. over a 4-hour period and the mixture was allowed to stir at that temperature for 6 hours. After cooling, the reaction mixture was poured into 2-3 times its volume of methanol to precipitate the reaction product. The precipitated reaction product was repeatedly ex-

## 5

tracted with methanol in a high-speed blender until trichlorobenzene was completely removed and was finally vacuum dried. The reaction product contained 1.8 weight percent phosphorus, 2.8 weight percent sulfur, and 1.1 weight percent nitrogen.

## EXAMPLE 2

## Preparation of additive

A reaction product containing 1.0 weight percent phosphorus, 1.5 weight percent sulfur, and 0.51 weight percent nitrogen was prepared using a mole ratio of 1/1/10 of the same terpolymer used in Example 1/P<sub>2</sub>S<sub>5</sub>/N,N-dimethyl-1,3-propanediamine ingredients under the same reaction conditions as described in Example 1.

## EXAMPLE 3

## Preparation of additive

A reaction product containing 2.4 weight percent phosphorus, 3.5 weight percent sulfur, and 1.8 weight percent nitrogen was prepared using a mole ratio of terpolymer (54% E/42% P/4.1% 1,4-HD and inherent viscosity of 0.44)/P<sub>2</sub>S<sub>5</sub>/N,N-dimethyl-1,3-propanediamine of 1/4/16 under the same reaction conditions of Example 1.

## EXAMPLE 4

## Preparation of additives

A reaction product containing 1 weight percent phosphorus, 1.4 weight percent sulfur, and 0.52 weight percent nitrogen was prepared using a mole ratio of terpolymer (59.7% E/37.9% P/2.4% 1,4-HD and inherent viscosity of 0.59)/P<sub>2</sub>S<sub>5</sub>/N,N-dimethyl-1,3-propanediamine of 1/1/10 under the same reaction conditions of Example 1.

## EXAMPLE 5

## Viscosity properties

This example shows that the reaction products of this invention possess the thickening properties required for use as a viscosity index improver in multigraded lubricating oils.

The products of Examples 1 and 2 were each added to refined 131 neutral oil S.U.S. at 100° F. to result in compositions containing 1, 2 and 3 percent by total weight. The thickening, as measured in terms of viscosity, resulting from the addition of the stated amounts of additive is shown in the following Table A:

TABLE A

| Additive                 | Wt. percent of additive present in oil | Viscosity of oil |             |       | ASTM slope |
|--------------------------|----------------------------------------|------------------|-------------|-------|------------|
|                          |                                        | Cs. at 210° F.   | p. at 0° F. |       |            |
| None.....                | 0                                      | 4.72             | 10.1        |       | 0.763      |
| Product of Example 1.... | 1                                      | 6.11             | 11.2        | 0.709 |            |
|                          | 2                                      | 8.48             | 13.1        | 0.667 |            |
|                          | 3                                      | 12.88            | 14.8        | 0.633 |            |
| Product of Example 2.... | 1                                      | 6.15             | 11.0        | 0.707 |            |
|                          | 2                                      | 8.35             | 12.8        | 0.669 |            |
|                          | 3                                      | 11.72            | 14.7        | 0.638 |            |

The measurement of cs. (centistokes) at 210° F. was carried out by ASTM Test Method D445.

The measurement of p. (poise) at 0° F. was measured using a cold cranking simulator. A universal motor, run at constant voltage, drives a rotor which is closely fitted inside a stator. A small portion of the oil/additive composition fills the space between the rotor and stator which are maintained at 0° F. The speed of the rotor is a function of, and is calibrated to determine the viscosity of the oil/additive composition in poises.

The slope was obtained by ASTM Test Method D341.

Table A shows that the additives of this invention, in an amount of 1 weight percent, increase the viscosity of the oil as measured in cs. at 210° F. by about 30 percent; while an amount of 3 weight percent increases the viscosity by about 170 percent.

## 6

## EXAMPLE 6

## Shear stability

The shear stabilities of oil compositions containing the same base oil as in the viscosity index test of Example 5 and the amount of various ethylene terpolymers necessary to increase the viscosity of the oil composition to 11.5±0.1 centistokes at 210° F. were determined using a 250 w., 10 kc. magnetostrictive sonic oscillator in accordance with the technique described in "Proposed Method of Test for Shear Stability of Polymer-Containing Oils," in ASTM Standards, vol. I, page 1160 (October 1961). The procedure was modified by shearing a 50 ml. sample for 60 minutes at 100° F. at 0.6 r.f. amps. Shear stability is expressed as the average percent retention of viscosity in centistokes at 210° F. and 100° F. The results are shown in Table B following:

TABLE B.—SHEAR STABILITY IN SONIC TEST

| Additive                  | Weight percent of additive required to thicken oil to 11.4 cs./210° F. | Percent viscosity retention |
|---------------------------|------------------------------------------------------------------------|-----------------------------|
| Product of Example 2..... | 2.9                                                                    | 99                          |
| Product of Example 1..... | 2.8                                                                    | 99                          |

Table B shows that the shear stability of the additives of this invention is substantially maintained.

## EXAMPLE 7

## Dispersancy power

Low temperature deposition tests in a single cylinder CLR engine for 180 hours according to the procedure of FTM-791a Method 348 Modified were carried out. Lubricating oil compositions labeled A, B, and C were tested. Each composition contained lubricating oil, zinc dialkyl-dithiophosphate and a high-base calcium sulfonate (each added to provide rust-inhibition and antioxidant properties to the oil). The ingredients of compositions A, B, and C are listed as follows:

| Ingredients                                     | A<br>(control) | B   | C   |
|-------------------------------------------------|----------------|-----|-----|
| SAE-30 base oil (618.8 S.U.S. at 100° F.).....  | (1)            | (1) | (1) |
| Zinc dialkyl-dithiophosphate, wt., percent..... | 1              | 1   | 1   |
| High-base calcium sulfonate, wt., percent.....  | 2              | 2   | 2   |
| Additive of Example 1, wt. percent.....         | 2              | 2   | 2   |
| Additive of Example 4, wt. percent.....         |                |     | 2   |

<sup>1</sup> Present.

The results are shown in Table C, as follows, in which a rating of 10 represents maximum cleaning of the piston skirt and a rating of 50 represents maximum cleaning of "Total" and of "CRC Sludge":

TABLE C.—RATINGS

| Composition                   | Varnish      |       | Percent clogging |                     |                   |
|-------------------------------|--------------|-------|------------------|---------------------|-------------------|
|                               | Piston skirt | Total | CRC sludge       | Oil screen, percent | Oil ring, percent |
| A <sup>1</sup> (control)..... | 6            | 35    | 37               | 30                  | 51                |
| B.....                        | 7.7          | 44    | 48               | 5                   | 18                |
| C.....                        | 8.0          | 37    | 44               | 10                  | 1                 |

<sup>1</sup> 10W-50 base oil (131 S.U.S. at 100° F.).

The results of Table C show that the oil additives of this invention improve dispersancy in low-temperature deposition tests.

## EXAMPLE 8

## Anti-rusting properties

The anti-rust properties of the additives of this invention were determined by placing 30 ml. of an oil blend of compositions A-C, described below, in 4-oz. jars along with 3 ml. of synthetic exhaust condensate and a SAE 1020 carbon steel billet. The mixture was heated for 24 hours at 140° F. The billet was removed, rinsed with a hydrocarbon solvent and examined for the percent area rusted.

The composition of the oil blends and the results obtained using them are shown in Table D as follows:

TABLE D

| Composition:                                                              | Percent area<br>rusted |
|---------------------------------------------------------------------------|------------------------|
| (A) 10W-50 base oil (131 S.U.S. at 100° F.)                               | Over 50                |
| (B) Base oil of A above and 2 weight percent of the additive of Example 4 | Less than 1            |
| (C) Base oil of A above and 2 weight percent of the additive of Example 1 | Less than 1            |

Table D clearly shows the anti-rust properties of the compositions of this invention.

## EXAMPLE 9

## Antioxidant and bearing corrosion inhibition properties

Products of this invention were evaluated for their lube oil antioxidant and bearing corrosion inhibition properties in the MacCoull Oxidation Test. The MacCoull Test is a method of determining the oxidation stability and corrosive effect of lubricating oils on a copper-lead bearing. The test, a modification of the method originally developed by The Texas Co. (Method SP-148-48, Feb. 1, 1948), is carried out so as to reproduce the oil-bearing conditions which actually exist in an engine, namely, circulation of the oil through a rotating bearing, contact with other metal surfaces and air, and recirculation through the bearing. The oil sample being tested is oxidized at a temperature of 350° F. After 10 hours of operation, each bearing weight is subtracted from its corresponding original weight. The difference, reported in milligrams, is known as the bearing weight loss. The degree of bearing corrosion by the oil is indicated by the amount of bearing weight loss, a non-corrosive oil showing little or no bearing weight loss and, conversely, a highly corrosive oil showing a much greater bearing weight loss.

The antioxidant properties were measured by the change in the total acid number before and after the test. Total Acid Number, Total Base Number, and Viscosity tests are run on the oil in order to obtain a measure of its resistance to oxidation. The relative increase in total acid number and viscosity, and the decrease in total base number are indicative of oxidation of the oil.

In the absence of any other additives in the oil blend, the products of this invention caused a decrease in the amount of oxidation of the oil, over the amount occurring in the oil with no additives in it. In the presence of other commercial anti-oxidants, the level is decreased even further, showing that there are no incompatibility problems to be concerned with. Another feature of the additives of this invention is that, in combination with a commercial antioxidant, zinc dialkyldithiophosphate and a high-base calcium petroleum sulfonate, a high percent of the basicity is retained. This indicates that the additives of this invention possess long detergent life.

The results obtained are described in Table E as follows:

## EXAMPLE 10

Antiwear properties ASTM Test Method D2670-67, Standard Method for measuring wear properties of fluid lubricants (Falex Method)

The Falex Wear test was used to evaluate the antiwear properties of the additives of this invention. In this standard load/wear test, the steel bushings were SAE 4615-4620, 90 minimum Rockwell B, 15 RMS maximum. The steel pen was Sanderson special drill rod, 98-102 Rockwell B, RMS maximum. In the Table F below, the oil compositions employed were mixtures of Solvent 131 SUS neutral and the additive indicated. The results are shown as follows:

15

TABLE F.—FALEX WEAR TEST

[Oil=Solvent refined neutral oil, 131 S.U.S. at 100° F.]

| Additive used                                                    | Load (lb.) at seizure | Wear at 1,000 lbs./60 min. |                 |
|------------------------------------------------------------------|-----------------------|----------------------------|-----------------|
|                                                                  |                       | Total, mg. <sup>1</sup>    | Scar width, mm. |
| None                                                             | 2,350                 | (1)                        | -----           |
| 1 wt. percent zinc dialkyldithiophosphate, a commercial additive | 1,400                 | 94.1                       | 1.25            |
| 2 wt. percent product of Example 2                               | 2,275                 | 0.8                        | 0.38            |
| 2 wt. percent product of Example 1                               | 2,600                 | 0.6                        | 0.38            |

<sup>1</sup> Seizure.

As shown by the table, the additives of this invention impart superior antiwear properties to the oil.

30

## EXAMPLE 11

Extreme pressure properties, Fed. Test Method Std. No. 791a, Method 6503, Dec. 30, 1961

Load-carrying capacity test (Mean-Hertz Load).—The terpolymer-P<sub>2</sub>S<sub>5</sub>-diamine additives of this invention were evaluated in a four-ball extreme pressure test. Since these additives exhibited very good antiwear properties, it was expected that they would also possess some Extreme Pressure properties. Frequently these two properties are found in the same additive. That was not the case with these products. The results of this test (Table G) show that they do not possess any Extreme Pressure properties in themselves. Surprisingly, however, when tested in combination with a commercial zinc dithiophosphate-type Extreme Pressure additive, the additives of this invention greatly enhance the Extreme Pressure properties of the zinc dithiophosphate additive, as shown by an increase in the Mean Hertz Load from 38 to 54 kilograms (in Table G). This synergistic effect was dependent upon the concentration of the zinc dithiophosphate. When the zinc dithiophosphate concentration was decreased from 1 to 0.5 percent, the Extreme Pressure properties decreased as well.

The test was carried out with a 10-second test duration at each applied load. The Mean Hertz Load is calculated from the series of scar diameters. The Point of Incipient Seizure is the highest load at which the scar diameter in-

TABLE E.—MACCOULL OXIDATION TEST (10 HOURS AT 350°F.)

Oil A=Solvent refined neutral oil 131 SUS at 100° F.

Oil B=Oil A + 1 wt. percent zinc dialkyldithiophosphate + 2 wt. percent high-base calcium sulfonate.

| Composition, oil plus additive<br>(2 wt. percent) | ASTM test method viscosity (D 445) |       |         |       | mg. KOH/g. |       |         |       | Bearing<br>wt. loss,<br>mg. |  |
|---------------------------------------------------|------------------------------------|-------|---------|-------|------------|-------|---------|-------|-----------------------------|--|
|                                                   | 210° F.                            |       | 100° F. |       | TAN-E      |       | TBN-E   |       |                             |  |
|                                                   | Initial                            | Final | Initial | Final | Initial    | Final | Initial | Final |                             |  |
| A plus none                                       | 4.76                               | 7.95  | 27.3    | 64.4  | .04        | 11.3  | 0       | 0     | 63                          |  |
| A plus product of Example 4                       | 9.41                               | 7.86  | 63.8    | 54.2  | 0.1        | 3.6   | 0.2     | 0     | 18                          |  |
| A plus product of Example 2                       | 8.01                               | 7.31  | 51.7    | 48.5  | 1.2        | 2.2   | 0.1     | 0     | 19                          |  |
| B plus product of Example 4                       | 9.93                               | 15.99 | 70.1    | 118.2 | 2.0        | 1.7   | 5.5     | 1.9   | 5                           |  |
| B plus product of Example 2                       | 8.18                               | 10.31 | 54.5    | 69.4  | 1.9        | 1.6   | 5.9     | 1.4   | 5                           |  |

The table shows that the presence of additives of this invention retards oxidation of the oil and reduces corrosion on bearings.

75 indicates that the oil is still functioning in the region of full fluid film lubrication. The scar diameters at loads above this point show the performance of the oil in the

area of thin film or boundary lubrication. The weld point is the load at which the four balls weld or at which the scar diameter exceeds 2.5 mm. The results are described in Table G, as follows:

TABLE G.—LOAD-CARRYING CAPACITY (FTM 791a  
METHOD 6503)  
[Oil-Solvent refined neutral oil 131 SUS. at 100° F.]

| Additive used in the oil                                                         | Weld point, kg. | Point of incipient seizure, kg. | Mean hertz load, kg. |
|----------------------------------------------------------------------------------|-----------------|---------------------------------|----------------------|
| None                                                                             | 71              | 40                              | 15.9                 |
| 1 wt. percent zinc dialkyldithiophosphate (A)                                    | 112             | 71                              | 38.2                 |
| 1 wt. percent (A) plus 2 wt. percent highbase calcium sulfonate (B)              | 141             | 63                              | 32.4                 |
| 2 wt. percent product of Example 4                                               | 79              | 50                              | 20.2                 |
| 2 wt. percent product of Example 1                                               | 71              | 40                              | 16.1                 |
| 1 wt. percent (A) plus 2 wt. percent product of Example 4                        | 112             | 79                              | 40.1                 |
| 1 wt. percent (A) plus 2 wt. percent product of Example 1                        | 158             | 112                             | 53.9                 |
| 0.5 wt. percent (A) plus 2 wt. percent product of Example 1                      | 178             | 79                              | 39.6                 |
| 1 wt. percent (A) plus 2 wt. percent (B) plus 2 wt. percent product of Example 1 | 158             | 100                             | 47.9                 |

The foregoing examples demonstrate that the terpolymer-P<sub>2</sub>S<sub>5</sub>-amine additives of this invention are truly multifunctional additives. They possess surprisingly good Viscosity Index improving properties. They also show an unexpected synergistic effect on extreme pressure properties when used with a commercial zinc dialkyldithiophosphate additive. In addition they have excellent low-temperature detergent, antioxidant, bearing corrosion inhibition, antirusting and antiwear properties. At an average use concentration of 2 wt. percent in the lubricating oil, the desired level of performance in each of the above properties can be achieved with only the single additive of the invention. This results in simplification for the refiner in formulating a complete crankcase lubricating oil. In addition, the additive is ashless.

The foregoing detailed description has been given for clearness of understanding only and no unnecessary limitations are to be understood therefrom. The invention is not limited to the exact details shown and described, for obvious modifications will occur to those skilled in the art.

The embodiments of the invention in which an exclusive property or privilege are claimed are defined as follows:

- 5 1. A lubricant additive consisting essentially of the product obtained by reacting  
(A) a phosphosulfurized ethylene/propylene/1,4-hexadiene terpolymer having an average molecular weight of between about 3,500 and about 65,000 and containing about 35-70 weight percent propylene, about 1-6 weight percent 1,4-hexadiene and the remainder being ethylene; with  
(B) an amine of the formula H<sub>2</sub>N-(CH<sub>2</sub>)<sub>x</sub>NRR<sub>1</sub> wherein x is an integer of 2 or 3, and R and R<sub>1</sub> are alkyl groups of 1-4 carbon atoms.
- 10 15 2. The additive of claim 1 in which the terpolymer contains 42-55 weight percent propylene, 1-4 weight percent 1,4-hexadiene with the remainder ethylene and in which the molecular weight is between about 3,500 and 35,000.
- 15 20 3. The additive of claim 2 in which the amine is N,N-dimethyl-1,3-propanediamine.
- 20 4. A lubricant additive concentrate comprising a lubricating amount of a neutral lubricating oil and about 5 to about 50% by weight of the additive of claim 1.
- 25 5. A lubricant composition comprising a lubricating amount of a mineral lubricating oil and from about 0.1 to about 4% by weight of the additive of claim 1.

#### References Cited

##### UNITED STATES PATENTS

- 30 2,800,467 7/1957 Garwood et al. ----- 260—139  
3,329,612 7/1967 Ferm et al. ----- 252—32.7X

##### FOREIGN PATENTS

- 35 1,537,571 4/1968 France ----- 252—59

35 DANIEL E. WYMAN, Primary Examiner

W. H. CANNON, Assistant Examiner

##### U.S. CL. X.R.

- 40 252—37.7; 260—139, 501.2